

July 11, 1933.

M. F. TUCKER

1,917,407

ELECTRICAL FUSE PLUG

Filed March 16, 1931

*Fig.1*

*Observation Window of Cellulose Acetate.*



*Fig.2.*



*Observation Window of Cellulose Acetate.*

Inventor,

*Milton F. Tucker;*

By

*Newton M. Perrine*

*Daniel J. Mayne*

## UNITED STATES PATENT OFFICE

MILTON F. TUCKER, OF PROVIDENCE, RHODE ISLAND, ASSIGNOR TO EASTMAN KODAK COMPANY, OF ROCHESTER, NEW YORK, A CORPORATION OF NEW YORK

## ELECTRICAL FUSE PLUG

Application filed March 16, 1931. Serial No. 522,935.

This invention relates to electrical fuse plugs having windows or observation orifice covers of cellulose acetate sheeting.

In the production of electrical fuse plugs it has been the practice for many years to place a window composed of a thin sheet of mica on the top of said plugs for the purpose of permitting observation to be made as to the condition of the fuse wire within the plug. While mica has been satisfactory from an electrical standpoint, it has shown many disadvantages with reference to the utility of such plugs, among which may be mentioned the low transmission of light through the mica and its high reflective power, as well as the great dispersion of light due to surface irregularities inherent in the highly developed cleavage which lepidolite, muscovite and other types of mica are known to possess. Also, because of its high cost, mica has been unsuitable for this purpose.

Recently fuse plugs have been manufactured containing glass windows but these fuse plugs have the disadvantage in commercial use of extreme brittleness which leads to many broken windows in plugs of this type both in handling and in use. In neither of the types of fuse plug windows mentioned above is there any means of ascertaining whether or not the fuse wire has been melted except by observation through the window which is usually unsatisfactory because of the deep recess in the plug in which the fuse wire is placed and the dark places in which fuse plugs are usually located in use.

I have found that cellulose acetate in sheet form of any desired thickness, for example, from .005 inches to .025 inches may be successfully employed as windows for fuse plugs. The cellulose acetate may contain admixed therewith plasticizers such as di-ethyl phthalate, ortho-cresyl-para-toluene-sulfonate, benzophenone, or other materials imparting similar properties to cellulose acetate. If desired, other plastic materials such as gums, waxes, heavy metal soap, solid fatty acids, or a material which will cause the cellulose acetate sheet to darken or blacken upon decomposition by heating such, for instance, as cinnabar, flowers of sulfur, selenium salts,

etc., chlorinated hydrocarbons, such as chlorinated diphenyl etc. may be added to the cellulose acetate, if desired. It is understood, of course, that the acetate itself will darken perceptibly due to hot metal which is thrown off by the fuse when being blown. I have found that the cellulose acetate sheet will withstand the action of heat caused by high current over considerable periods of time before the fuse is blown. I have also found that acetate sheets are much more transparent than mica when used in a similar situation, and that upon blowing of the fuse the cellulose acetate sheet darkens or blackens over all or a portion of its inside surface, in this way giving easily visible evidence that the fuse has been blown.

As an example of the value of cellulose sheets for the purpose disclosed in the above paragraph, a 20 ampere fuse plug was supplied with a window composed of a sheet of cellulose acetate .010 inches thick, which acetate contained 16% of the weight of the cellulose acetate as ortho-cresyl-para-toluene-sulfonate. When a current of approximately 40 amperes was run through this plug, the fuse wire melted very rapidly and "spattered" with considerable force, but the cellulose acetate window was quite unimpaired except that it had darkened quite perceptibly.

In another instance two fuse plugs of the same 20 ampere rating were maintained at approximately 18 amperes for nearly two hours, during which time they reached a temperature of 150° F. and even higher. The current was then increased to 25 amperes and the fuse wire melted in one instance 25 minutes after the current had been increased, and the second in 35 minutes. These fuses, after the fuse wire had melted, showed an unmistakable mark on the inner surface of the cellulose acetate window. Before the fuse wire had melted, the cellulose acetate window had shown much better light transmission than either the mica or the thick glass windows in similar plugs mentioned above. After the fuse wire had melted, the surface of the cellulose acetate window bore a mark produced by imbedding a portion of the molten metal of which the fuse wire was com-

posed into the cellulose acetate window. This resulted in some plastic flow of the inner surface of the window as well as surface decomposition of the cellulose acetate so affected, darkening the acetate sheet in that locality giving an unmistakable signal of the blowing of the fuse.

In the accompanying drawing in which like reference numerals refer to like parts, 10 a fuse plug is illustrated having a cellulose acetate window. Fig. I is a vertical section taken through the center of the fuse plug and Fig. II is a plan view thereof. The fuse plug is composed of the base or foundation 1 on which are located the terminals 2 and 3. Connecting these terminals is the fuse wire 4, with the customary area of high resistance. The window 5 composed of cellulose derivative sheeting is held to the foundation 15 of the plug by means of the annular ring 6.

It is understood that any thickness of sheet desired which admits of transparency may be used. However, for reasons of economy it 25 is preferred that the sheeting be only thick enough to form a window which is fairly 30 resistant to handling.

Other fatty acid esters, of cellulose, especially the higher fatty acid esters or the 35 mixed esters such as cellulose acetate-propionate, cellulose propionate-stearate, cellulose acetate-benzoate, cellulose butyrate etc., or cellulose ethers such as ethyl cellulose may be used in this connection. Nitro-cellulose can also be used, but it has the disadvantages of high inflammability and of 40 possible darkening on long standing.

What I claim as my invention and desire to secure by Letters Patent of the United 45 States is:

1. An electrical fuse plug having an observation window of cellulose organic derivative sheeting in proximity to the fuse wire of the fuse plug.

2. An electrical fuse plug having an observation window of cellulose mixed organic ester sheeting in proximity to the fuse wire of the fuse plug.

3. An electrical fuse plug having an observation window of cellulose higher organic ester sheeting in proximity to the fuse wire of the fuse plug.

4. An electrical fuse plug having an observation window of cellulose acetate sheeting in proximity to the fuse wire of the fuse plug.

5. An electrical fuse plug having an observation window which comprises a cellulose derivative and a material which darkens upon the blowing of the fuse.

6. An electrical fuse plug having an observation window which comprises cellulose acetate and a material which darkens upon the blowing of the fuse.

7. An electrical fuse plug having an observation window comprising cellulose acetate and a plasticizer.

8. An observation window for an electrical fuse plug comprising cellulose derivative sheeting which darkens at the temperature 95 of melting of the fusible alloy.

9. An observation window for an electrical fuse plug comprising cellulose acetate and a material which darkens upon heating.

Signed at Providence, R. I. this 9th day of 10 March 1931.

MILTON F. TUCKER.